

Dec. 25, 1945.

J. V. CARON

2,391,615

## METHOD OF MAKING HEAT INTERCHANGE APPARATUS

Filed Aug. 25, 1942



Inventor  
Joseph Victor Baron  
Knight Brown (Purinby May)

## UNITED STATES PATENT OFFICE

2,391,615

## METHOD OF MAKING HEAT INTERCHANGE APPARATUS

Joseph Victor Caron, Haverhill, Mass.

Application August 25, 1942, Serial No. 455,985

8 Claims. (Cl. 22—193)

This invention relates to the manufacture of heat interchange apparatus, such, for example, as internal combustion engines and compression cylinders and the like, and more particularly where the heat interchange is produced by providing relatively thin fins projecting from a cylinder or the like about which a current of air or other gas is caused to flow.

It is well known that certain metals are much more efficient as heat conductors than others, copper being one of the best, but copper is not well suited to withstand heavy pressures, and it also has a high coefficient of thermal expansion and is relatively soft. Air cooled pressure cylinders are commonly made of ferrous material, often of cast iron, but it is difficult to form cooling fins of this material sufficiently close together and sufficient thin, and yet strong, to be suitable wherever much heat is to be dissipated, and because iron or other ferrous material is much inferior to copper in heat conductivity.

For these reasons it has become customary to deform engine and compressor cylinders as steel or alloy forgings and then to cut slots inwardly, leaving integral fins between the cuts. This is an expensive procedure and the fins being made of the steel or alloy are inferior in heat conducting qualities to copper fins.

It has been attempted, therefore, to pre-form fins of copper or alloys of copper and to cast a cylinder or the like so as to embed the inner peripheral portions of said fins in said cylinder or the like while said fins are held in proper relation, so as to project from the cast cylinder or the like. This, however, entails certain serious problems and so far as I am aware has never been done successfully on a commercial scale, and particularly when using copper fins.

In accordance with the present invention, however, this may be done commercially and when the teaching of this invention is carefully followed, with relatively small rejections on account of imperfect casting. By so doing, no machining of the outside of the cylinder or block to produce fins is required, and if desired the head may be formed integral with the cylinder thus avoiding the necessity of machining and securing these parts together. It will be noted that the molten iron when cast will have a temperature in the neighborhood of 2800° F. and the melting point

of copper is much lower, around 1950° F., so that when a mass of this molten iron contacts with the preformed copper fins, unless the heat from the iron can be quickly dissipated, it will melt off the copper portion with which the molten

iron contacts. While surface melting and fusion is essential in order to effect a welding of the fin and body portions together so that heat conductivity between them when in use may be rapid, this must not be allowed to go so far as to melt off the copper contacted by the molten iron from the remainder of the copper element. The application of this method to copper fins for cast iron cylinders is a most important one, but this invention is also applicable to other situations where it may not be desired to use metals having such different melting points as copper and cast iron. For example, in some cases sufficient cooling may be afforded by the use of soft steel fins projecting from a cast iron cylinder, or there may be other combinations of alloys such as the aluminum and magnesium alloys now employed for internal combustion aircraft or other engines for the cylinders and cylinder heads.

For a more complete understanding of this invention, reference may be had to the accompanying drawing in which

Figure 1 is a perspective view of a cast two-cylinder L head internal combustion engine block provided with sheet metal cooling fins and made in accordance with this invention.

Figure 2 is a perspective view of a two-part pattern for the barrel portion of a single cylinder block, the parts of the pattern being slightly separated.

Figure 3 is a perspective view showing a two-part sheet metal fin.

Figure 4 is a fragmentary vertical section through a flask and mold showing the pattern of Figure 2 and fins like the showing of Figure 3 in position therein.

Figure 5 is a view similar to Figure 4, but showing the pattern removed and the core in place, the mold being ready for pouring.

Figure 6 is a cross-sectional view on line 6—6 of Figure 5.

Figures 7 and 8 are fragmentary sectional views similar to portions of Figures 4 and 5 but showing a modification wherein the fins are closely spaced.

Figure 9 is a fragmentary side elevation of a cylinder for a valve in head engine and finned in accordance with this invention.

Figure 10 is an elevation of a single cylinder having an integral head.

In Figure 1 of the accompanying drawing is shown two cylinders cast in a block for an L head internal combustion engine. These will ordinarily be cast in two sections, one comprising the barrels of the cylinders and the hous-

ing for the valves and some of their actuating mechanism, and the other section comprising the cylinder heads 3. These two portions are secured together as by bolts 4. These two parts, as shown, are provided with cooling fins, those on the barrel 1 and the valve housing 2 being arranged parallel to each other around the circumferences of these parts, while the fins on the head are arranged laterally and in line with the air currents which will pass across the engine during operation. These fins in accordance with the present invention may well be formed of sheet metal of any desired composition.

In Figure 2 is shown a pattern for the barrel of a single cylinder. This pattern is formed in upper and lower parts 10 and 11, each of which is provided at its ends with the core prints 12 and 13 which are of smaller external diameter than the remainder of the pattern. Along the barrel portion of the pattern there are provided outwardly projecting parallel beads or ribs 15 which may be substantially semi-cylindrical in outline, these being arranged spaced apart in accordance with the desired spacing of the fins. Each of these beads is provided with a central groove 16 of sufficient size to admit the inner edge of the pre-formed fin, such as is shown detached in Figure 3. These fins are formed as annular half sections to correspond with the halves of the pattern and they may be well formed of sheet metal of the particular material desired for cooling. For example, in the body of the cylinder they may be formed of soft steel, or if greater cooling effect is desired, they may be formed of copper. Preferably they are formed with perforations as at 17, it being found in practice that such perforations tend to cause more effective cooling action of the air which comes in contact with the fins. They also may serve a desirable purpose in assembling the pattern with the fins thereon in the mold as will later appear.

The fins are assembled on the pattern parts with their inner edges inserted in the grooves 16 of the beads 15, and rods or bars 18 inserted through aligned holes 17 may be employed to facilitate assembly of these parts. The two parts of the pattern with the fins and rods or bars thus assembled therewith are then employed to make a green sand mold in the cope and drag of the flask in the well known manner. These fins and the rods or bars remain in the green sand mold but said rods or bars are removed from the fins after the casting operation and after the castings are taken from the mold.

The method of molding a plurality of cylinders in block is the same as for individual cylinders, except that the fins may be continuous for the full number of cylinders but made in halves, one half for each part of the pattern.

Where the fins are made of copper it may be found desirable to employ molding sand somewhat more moist than in the ordinary practice of casting iron, but this should not be sufficiently moist to cause blowing of the casting during pouring. However, due to the high conductivity of the copper, such additional moisture provides additional cooling effect to the fins, helping to prevent them from becoming melted off by the great heat of the molten iron, the melting temperature of which is considerably higher than that of the copper.

When the pattern is drawn from the green sand mold, the fins are left embedded in said mold, with their inner edges projecting into the

recesses 19 in the outer wall of the mold cavity 20, these recesses having been formed by the presence of the beads 15 of the mold. When the core 21 is now placed in position and the mold 5 reassembled, said mold is ready for pouring. The recesses 19 in the outer wall of the mold cavity form beads in the cast cylinder corresponding to the pattern beads, within which the inner projecting edges of the fins are embedded, and these beads thus form restricted masses of the molten metal which are cooled rapidly by the heat conducted away therefrom by the fins so that they become cooled and solidified earlier than the mass of the metal in the main mold cavity 20. Thus the fins 15 are not subjected to the full action of the high temperatures of the molten metal of the whole mass, this further acting to prevent the fin edges from becoming melted off from the remainder of the fins during the casting operation. By reason 10 of the spaces between the beads, the weight of the cylinder is also reduced.

It is also important that the mold be filled during the casting operation in such a manner that the flow of molten metal takes place along 25 the side faces of the projecting portions of the fin rather than crosswise thereof, as any cross flow would tend to wash off the projecting portions of the fins and thus destroy their attachment to the cast cylinder. This may be done by 30 providing sprue holes such as 25 which extend down to the lower portion of the drag 11 and are gated to the mold cavity 20 from beneath as at 26, the mold also being provided with suitable 35 risers as 27 to provide vents and insure that the mold cavity is entirely filled through the hydrostatic pressure of the molten metal in the mold. With this arrangement the molten metal rises from the bottom of the mold cavity upward in line with the fins, and the mold should be poured 40 from a sufficient number of points so as to insure even heat distribution throughout the mold cavity.

In some instances it may be found desirable to space the fins very closely for additional cooling 45 effect, as, for example, in the combustion chambers of internal combustion engine cylinder heads. Where this is desired it may be unnecessary to employ the projecting beads within which the inner edges of the fins are embedded even if there 50 were room for such beads, this being for the reason that with the increased number of fins in a given space, the heat conduction is so rapid that the surface portion of the casting is sufficiently quickly chilled as to prevent the possibility 55 of the fins being melted off by the mass of metal. Such an arrangement is shown in Figures 7 and 8, Figure 7 showing the pattern 30 being provided with grooves 31 to receive the fins 32, the depths of these grooves defining the amounts by which 60 the edges of the fins will project into the mold cavity 28 of the mold as shown in Figure 8. This arrangement of the fins corresponds to the showing of Figure 9 for the combustion chamber portion of a valve in head engine. This particular 65 arrangement of the fins is not claimed herein, but forms subject matter of a companion application.

Even when soft steel fins are employed, as for 70 the barrel of a cylinder, the formation of ribs on the pattern may be found desirable, as due to the less conductivity of the steel than the copper, these bead portions of the casting retain sufficient heat to effect the desired welding of the soft steel to the cast iron of the completed cylinder. For 75 cylinders, say, of a diameter of four inches and

wall thickness of  $\frac{1}{16}$  inch, beads  $\frac{3}{2}$  of an inch in diameter grooved to a depth of  $\frac{3}{32}$  of an inch, and copper fins of a thickness .015 inch, one inch in width and arranged five to each inch of cylinder length, will ordinarily be found satisfactory. With larger or smaller sizes of cylinders, the proportions will, of course, be modified accordingly, but with this as a guide the skilled foundryman should find no difficulty in proper proportioning the parts to insure welding of copper fins to cast iron and without melting off the copper fins. If lighter weight cylinders are desired semi-steel or the lighter weight alloys may be substituted for the cast iron with appropriate changes in other factors.

In cases where very thin fins are desirable, they may be protected from being melted off by the molten cast iron by coating them previous to casting in the mold with protective compounds which act to delay actual contact of the molten iron with the fins and thus delay the full application of the heat from the molten iron to said fins, but do not prevent sufficient ultimate contact to prevent the desired welding of the fins to the cast iron. For example, such a composition may be formed of lead oxide, together with about a third as much graphite mixed with a heat-resistant oil, or fire clay, with or without graphite, and mixed with water or oil, may be used. The amount of such a composition to be added in any particular case may be determined by experimentation, it being understood, however, that considerable leeway is permissible while obtaining good results, and when determined for one particular set of conditions may be readily duplicated for the same conditions. Likewise the amount of moisture of the sand mold, which in the case of copper fins is preferably somewhat greater than in usual iron foundry practice, having once been determined, may be maintained satisfactorily. Here, again, there is considerable leeway, provided the pouring temperatures are maintained substantially uniform as may be done in commercial foundry practice.

In Figure 10 is shown a single cylinder with integral head and provided with fins 35 cast in in accordance with this invention on both the cylinder side wall and the head.

From the foregoing description of this invention it should be understood that various other modifications and changes may be made without departing from the spirit or scope of this invention.

I claim:

1. In a method of manufacturing a finned body with the aid of a molding flask having a drag and a cope; the steps of constructing a plurality of semi-circular fin halves; forming a green sand mold section in said drag with half the number of said fin halves embedded in said mold section and projecting into the mold cavity; forming a second green sand mold section in said cope with

the remainder of said fin halves embedded in this mold section and projecting into the mold cavity; assembling said green sand mold sections, with the fin halves held by one section in end-to-end abutting relation with the fin halves held by the other section; pouring molten metal into the complete fin-holding mold; and removing said mold, leaving the cast body with attached fins.

2. In a method of manufacturing a finned body with the aid of a molding flask having a drag and a cope; the steps of constructing a pattern divided into a drag half and a cope half and having circumferential grooves; constructing a plurality of semi-circular fin halves; placing the inner peripheral edge portions of half the number of said fin halves in the grooves of said drag half of said pattern; placing the inner peripheral edge portions of the remainder of said fin halves in the grooves of said cope half of said pattern; with the aid of said drag, said drag half of said pattern, and the fin halves carried by the latter, forming a green sand mold section; with the aid of said cope, said cope half of said pattern, and the fin halves carried by the latter, forming a complementary green mold section; withdrawing said pattern halves from said green mold sections and the fin halves embedded therein, leaving said fin halves with their inner peripheral edge portions projecting from said green sand mold sections into the mold cavities thereof; assembling said green sand mold sections with the fin halves held by one section in end-to-end abutting relation with the fin halves held by the other section; pouring molten metal into the mold; and removing said mold, leaving the cast body with said fins attached thereto.

3. In a method of manufacturing a finned body with the aid of a molding flask having a drag and a cope; the steps of constructing a plurality of semi-circular fin halves; supporting half the number of said fin halves in said drag in spaced relation with each other; packing green sand in said drag and between the fin halves therein to form a green sand mold section in said drag with said half the number of said fin halves embedded in said mold section and projecting into the mold cavity; supporting the remainder of said fin halves in said cope in spaced relation with each other; packing green sand in said cope and between the fin halves therein to form a second green sand mold section in said cope with said remainder of said fin halves embedded in this mold section and projecting into the mold cavity; assembling said green sand mold sections and placing said fin halves held by one section in end-to-end abutting relation with said fin halves held by the other section; pouring molten metal into the complete fin-holding mold; and removing said mold, leaving the cast body with attached fins.

JOSEPH VICTOR CARON.